

Patented Aug. 8, 1950

2,517,958

# UNITED STATES PATENT OFFICE

2,517,958

## INORGANIC COMPOSITION FOR INHIBITING SAP STAIN

Leslie R. Bacon and Dwight B. Conklin, Wyandotte, Mich., assignors to Wyandotte Chemicals Corporation, Wyandotte, Mich., a corporation of Michigan

No Drawing. Application June 9, 1948,  
Serial No. 32,046

6 Claims. (Cl. 167—38.5)

1

The present invention relates to a chemical composition for preventing or inhibiting sap stain and mold growth in green wood and lumber. Sap stain, often times alternatively referred to as "blue stain," is a bluish or blue blackish discoloration within the body of the wood. It is caused by the growth of fungi, one of the most prominent of which is the species *Ceratostomella pilifera*. Sap stain is to be differentiated from mold growths which occur on the surface of the wood and which vary widely in color according to the characteristics of the several organisms which may develop.

A great many chemical compositions for inhibiting sap stain or mold growth in green wood have heretofore been devised. However, in most cases it has been found that such compositions were not capable of inhibiting both sap stain and mold growth.

Such prior chemical compositions have been based on both organic and inorganic chemicals, such as chlorophenolic compounds, organo-mercury compounds and sodium alkaline salts such as sodium carbonate, sodium bicarbonate and borax. Although the inorganic alkaline compounds have been used as sap stain inhibitors for more than the past forty years, they have been subject to the defect that they often stimulate rather than retard surface mold growths.

We have discovered that inorganic sap stain compositions containing a sodium borate, such as borax or sodium metaborate (i. e. sodium borate in which the  $\text{Na}_2\text{O}/\text{B}_2\text{O}_3$  mol ratio lies within the range of 1 to 1-2) and magnesium silicofluoride, overcome this previous defect, and quite to the contrary of what might be expected, successfully prevent rather than stimulate surface mold growths, as well as effecting excellent sap stain control.

The compositions of our invention are preferably employed by being made up in an aqueous solution of 5-25 pounds of composition per 100 gallons of water. The green wood or lumber to

be treated is then dipped or immersed in such aqueous solution and after dipping, stacked in the customary manner in the lumber yard and allowed to air dry for the usual period of three or four months.

Exemplary formulations embodying the principle of our invention are as follows:

|    | Ingredients                                                      | Per Cent by Weight, Solids Basis |
|----|------------------------------------------------------------------|----------------------------------|
| 10 |                                                                  |                                  |
| 15 | Magnesium Silicofluoride.....<br>Borax or Sodium Metaborate..... | 25-65<br>35-75                   |

Compositions made according to the above stated formulation ranges were made up and subjected to the following test:

- 20 Test specimens of Southern yellow pine in the form of circular blocks transversely cut from the sapwood of young trees were inoculated with a viable culture of the fungus *Ceratostomella pilifera*. Four of such specimen blocks were used 25 for each test composition. The test compositions were made up into aqueous solutions in the concentration as noted and applied to the fungus-inoculated blocks. Blocks were then maintained at a temperature of 82° F. and approximately 30 100% relative humidity for an incubation period of five weeks. At the end of such five weeks period, the area of sapwood stained on both the top and bottom surfaces of the four test blocks was measured and the average thereof noted. As 35 a control and for the purpose of comparison with a heretofore successful organic type of inorganic chemical compound composition, the borax-modified soda-sodium pentachlorophenate composition of U. S. Patent No. 2,392,987 was also employed 40 in the test series. Observations were made as to the degree of mold growth on the surface of the blocks. These test results are tabulated as follows:

| Compositions                                                                | Ingredients, Per Cent By Weight, Solids Basis | Per Cent Concentration in $\text{H}_2\text{O}$ Solution | Average Per Cent Sapwood Stained | Degree of Mold Growth |
|-----------------------------------------------------------------------------|-----------------------------------------------|---------------------------------------------------------|----------------------------------|-----------------------|
| Water Control.....                                                          |                                               |                                                         | 100.0                            | Medium.               |
| No. 1 (Control).....                                                        |                                               | 0.625                                                   | 100.0                            | None.                 |
| Borax.....                                                                  | 50.                                           |                                                         |                                  |                       |
| Modified Soda.....                                                          | 30.                                           |                                                         |                                  |                       |
| Sodium Pentachlorophenate.....                                              | 20.                                           |                                                         |                                  |                       |
| No. 2 (Control).....                                                        | Same as above.....                            | 1.250                                                   | 68.1                             | Do.                   |
| No. 3:.....                                                                 |                                               |                                                         |                                  |                       |
| Magnesium Silicofluoride<br>( $6\text{H}_2\text{O}$ ).....                  | 58.0.....                                     | 0.863                                                   | 0.0                              | Medium.               |
| Borax ( $\text{Na}_2\text{B}_4\text{O}_7 \cdot 10\text{H}_2\text{O}$ )..... | 42.0.....                                     |                                                         |                                  |                       |
| No. 4:.....                                                                 |                                               |                                                         |                                  |                       |
| Magnesium Silicofluoride<br>( $6\text{H}_2\text{O}$ ).....                  | 33.0.....                                     | 3.0                                                     | 0.0                              | None.                 |
| Sodium Metaborate<br>( $\text{NaBO}_3 \cdot 4\text{H}_2\text{O}$ ).....     | 67.0.....                                     |                                                         |                                  |                       |

It will be noted that the ingredients in the exemplary test compositions in the foregoing table are in the hydrated form. Magnesium silicofluoride, borax and sodium metaborate, are most ordinarily available on the market as hydrated rather than anhydrous salts. Our invention however is equally well operable when one or more of the ingredients are employed in the anhydrous form. Thus, in the appended claims, the definition of the ingredients of the composition should be understood as including the hydrated and anhydrous forms as equivalents.

Equivalent modes of practicing our invention may be followed provided that they are within the scope and purview of the appended claims.

We, therefore, distinctly claim and particularly point out as our invention:

1. A composition for inhibiting sap stain and mold growth in green wood comprising a mixture of magnesium silicofluoride and a sodium borate having an  $\text{Na}_2\text{O}/\text{B}_2\text{O}_3$  mol ratio of 1 to 1-2.
2. A composition for inhibiting sap stain and mold growth in green wood comprising a mixture of 25-65% by weight magnesium silicofluoride and 35-75% of a sodium borate having an  $\text{Na}_2\text{O}/\text{B}_2\text{O}_3$  mol ratio of 1 to 1-2.
3. A composition for inhibiting sap stain and mold growth in green wood comprising a mixture of approximately 58% by weight magnesium silicofluoride and 42% borax.
4. A composition for inhibiting sap stain and mold growth in green wood comprising a mixture

of approximately 33% by weight magnesium silicofluoride and 67% sodium metaborate.

5. An aqueous solution bath for treating green wood to inhibit sap stain and mold growth comprising 5-25 pounds per 100 gallons of water of the composition of claim 3.

6. An aqueous solution bath for treating green wood to inhibit sap stain and mold growth comprising 5-25 pounds per 100 gallons of water of the composition of claim 4.

LESLIE R. BACON.  
DWIGHT B. CONKLIN.

#### REFERENCES CITED

15 The following references are of record in the file of this patent:

#### UNITED STATES PATENTS

20 Number Name Date  
2,392,987 Hill Jan. 15, 1946

#### FOREIGN PATENTS

Number Country Date  
800,411 France May 4, 1936  
25 102,457 Australia Nov. 8, 1937

#### OTHER REFERENCES

Lindgren, "Prevention of Sap Stain and Mold in Southern Woods by Chemical Treatment," reprint from Southern Lumberman, Nashville, Tenn., Feb. 1, 1931, page 2 of reprint.